

# United States Patent [19]

Shen et al.

[11] 3,901,831

[45] Aug. 26, 1975

[54] **METHOD OF MAKING DENSE DETERGENT GRANULES** 3,639,289 2/1972 Heymer et al. .... 252/527 X

[75] Inventors: **Chung Y. Shen; Clayton F. Callis,**  
both of St Louis, Mo.

*Primary Examiner*—Benjamin R. Padgett

*Assistant Examiner*—E. Suzanne Parr

*Attorney, Agent, or Firm*—T. N. Wallin; J. E. Maurer;  
N. E. Willis

[73] Assignee: **Monsanto Company**, St. Louis, Mo.

[22] Filed: **Aug. 24, 1973**

[21] Appl. No.: **391,367**

[52] U.S. Cl. .... **252/527**; 23/313; 252/135;  
252/383; 252/546; 252/DIG. 11

## ABSTRACT

[51] Int. Cl.<sup>2</sup> .... **C11D 3/066**; C11D 3/07

[58] Field of Search .... 252/527, 546, 383, 384,  
252/385

Dense, free-flowing composite detergent additive granules are prepared by contacting hot inorganic salts such as sodium tripolyphosphate with aqueous alkali metal nitrilotriacetate under controlled conditions.

## [56] References Cited

### UNITED STATES PATENTS

3,620,979 11/1971 Corliss et al. .... 252/385

6 Claims, No Drawings

**METHOD OF MAKING DENSE DETERGENT  
GRANULES**

**BACKGROUND OF THE INVENTION**

This invention relates to a novel method of making composite detergent additive granules containing alkali metal nitrilotriacetate and an inorganic salt.

It is generally recognized that alkali metal nitrilotriacetates in combination with other inorganic salts such as sodium tripolyphosphate (hereinafter referred to as STP) exhibit excellent performance as detergency builders.

It is desirable to combine the nitrilotriacetate and inorganic salts in the form of composite granules to avoid the problems of segregation, stratification and non-homogeneity that are inherent when the constituents are dry blended. In some applications, such as machine dishwashing compositions, it is especially desirable to form very dense (at least 0.8 g/cc bulk density) composite granules in order that an effective quantity of detergent will be present within the limited volume of the detergent compartment of the machine dishwashing apparatus.

Conventional methods of making composite granules fail to provide the desired density and, in many instances, result in degradation of the composite constituents. For example, in conventional spray drying procedures, a wet slurry of the detergent components is sprayed into a stream of hot gases. This method, however, in volatilizing water from the particles formed, yields low density granules. In the case of STP-nitrilotriacetate spray-dried mixtures, the resultant composite bulk density is normally no more than 0.5 g/cc, which falls short of the 0.8 g/cc minimum density generally required for machine dishwashing applications. In addition, spray drying procedures yield an undesirably high level of decomposed alkali metal nitrilotriacetate, and sodium tripolyphosphate.

Another conventional method of preparing these dense composite granules is to dampen a mixture of the constituents to cause agglomeration and heat to a temperature of above 100°C to dry the granules formed. Although this procedure produces somewhat denser granules, the bulk density is still below the 0.8 g/cc required. The process is further disadvantageous if STP is present because it then results in hydrolytic degradation of the STP to less polymerized forms of phosphate.

Accordingly, the need for a method of making dense composite granules without excessive degradation of the constituents is well recognized by those skilled in the detergent art.

**SUMMARY OF THE INVENTION**

It is an object of the present invention to provide a method of making dense composite granules without excessive degradation of the ingredients thereof.

Basically, these objects are fulfilled by adding aqueous alkali metal nitrilotriacetate onto a hot agitated bed of inorganic salt under critically controlled conditions as hereinafter explained. The invention will be better understood from the following description of the preferred embodiments.

**DESCRIPTION OF THE PREFERRED  
EMBODIMENTS**

The process of this invention comprises adding aque-

ous alkali metal nitrilotriacetate to a hot agitated bed of inorganic salt.

The aqueous nitrilotriacetate can be an aqueous solution or slurry of disodium or trisodium, nitrilotriacetate, or mixtures thereof. The use of trisodium nitrilotriacetate is especially preferred in view of its availability and excellent detergency builder characteristics. The concentration of the nitrilotriacetate in the aqueous mixture should be from 40 to 70% by weight in order to provide a final product containing the amount of nitrilotriacetate desired for various detergency applications.

The inorganic salt to which the nitrilotriacetate is added can be sodium meta silicate, sodium carbonate, sodium sulfate, or mixtures thereof, sodium tripolyphosphate, or mixtures of sodium tripolyphosphate and sodium sulfate.

In the practice of the process the inorganic salt bed is heated to a temperature of from about 300°C to about 550°C prior to addition of the aqueous nitrilotriacetate. It is critical that this initial temperature be controlled within the above prescribed range because use of initial bed temperatures below about 300°C will not permit optimum rates of volatilization of water, and because use of temperatures above 550°C will cause undesirably excessive degradation of the nitrilotriacetate. The bed is agitated to effect uniform and homogenous mixing of its contents. Agitation of the bed can be effected by conventional stirring, shaking, vibrating or similar apparatus.

In a particularly preferred embodiment of this invention, STP is fed to the bed directly from a calciner. Since STP is conventionally manufactured in a calcining operation at temperatures of from 400°-500°C, the STP can be directly employed in the present invention without a costly heating or cooling step. Accordingly, this embodiment affords the advantage of significant cost savings.

Sufficient aqueous nitrilotriacetate is added to the bed of salt to provide a composite containing from about 3% to about 20% of the nitrilotriacetate. The aqueous nitrilotriacetate is preferably heated to a temperature of between 80°C and 110°C, prior to addition to the bed to facilitate rapid vaporization. However, the initial temperature of the aqueous nitrilotriacetate can be as low as 0°C or as high as 120°C if desired.

In adding the aqueous nitrilotriacetate to the inorganic salt two limitations must be observed. With respect to the following discussion of these limitations, the "bed temperatures" refer to the average temperature of the mass of inorganic salt to which aqueous nitrilotriacetate is being added.

First, the temperature of the composite bed to which the nitrilotriacetate is added must be below 300°C before the bed is permitted to dry. That is, when adding aqueous nitrilotriacetate to a bed having an initial temperature at or above 300°C, sufficient aqueous nitrilotriacetate must be added to lower the temperature below 300°C prior to vaporization of all the water added. Evolution of water from the bed will, therefore, be continuous during the period when aqueous nitrilotriacetate is added at temperatures above 300°C. If the bed is allowed to become totally dry (as evidenced by no evolution of steam) at temperatures above 300°C, excessive decomposition of the nitrilotriacetate will result.

Secondly, addition of the aqueous nitrilotriacetate and vaporization of the water contained therein must be complete (particle moisture content less than 1% by weight) before the bed temperature is below 160°C when STP is present or below 120°C when STP is not present. That is, the bed temperature, at which the evolution of steam from the bed ceases, must be above 60°C or 120°C. If, in the presence of STP, the addition continued or steam is being emitted from any section of the bed after that section has cooled to below 160°C, then the water in the presence of the STP will cause hydrolytic reversion of the STP to undesirable phosphates  $\text{Na}_5\text{P}_3\text{O}_{10} + \text{H}_2\text{O} \rightarrow \text{Na}_3\text{HP}_2\text{O}_7 + \text{NaHPO}_4$ . Note that when STP is not present in the bed, temperatures as low as 120°C can be used since hydrolytic degradation is not a problem. A temperature of at least 120°C is required to effectively dry the constituents.

The following specific examples are given in order to further explain and illustrate this invention. However, they are not intended to limit the scope in any way. In the examples, all parts and percentages are by weight unless otherwise indicated.

#### EXAMPLE I

Powdered sodium tripolyphosphate (analysis: 92% tripolyphosphate; 7% pyrophosphate; 1% trimetaphosphate) heated to 500°C is discharged into a screw conveyor to form an agitated bed.

An aqueous slurry containing 45% nitrilotriacetate is heated to 100°C and sprayed onto the bed continuously for about five minutes. This results in addition of 28.2 parts solution per 100 parts sodium tripolyphosphate. During addition of the solution to the bed, steam evolution is continuous indicating that the bed is not dehydrated at any time during solution addition. The bed temperature upon completion of solution addition and dehydration (particle moisture content less than 0.5%) is 200°C.

This procedure produces a granular composite product having particle sizes between -20 and 100 U.S. standard Mesh and a bulk density of about 0.92 ms/cc. The particles contain 11.21% trisodium nitrilotriacetate corresponding to the amount of nitrilotriacetate added and indicating substantially no degradation thereof. The analysis of sodium tripolyphosphate in the product particles is substantially identical to the analysis of the sodium tripolyphosphate added indicating absence of hydrolytic degradation in the process.

#### EXAMPLE II

The procedure of Example I is repeated except that

additional aqueous nitrilotriacetate is added until the bed temperature is 150°C. The assay of sodium tripolyphosphate in the product particles is only 85% with correspondingly higher percentages of pyro- and ortho-phosphates indicating that substantial hydrolytic degradation takes place when the limitations of the invention, as previously discussed, are not observed.

#### EXAMPLE III

The procedure of Example I is repeated except that less aqueous nitrilotriacetate is added and, upon completion of addition and bed dehydration, bed temperature is 325°C.

Product analysis indicates substantial degradation of the nitrilotriacetate added.

What is claimed is:

1. A method of making composite detergent additive granules containing from 3% to 20% alkali metal nitrilotriacetate the balance of said granules being an inorganic salt selected from the group consisting of sodium metasilicate, sodium carbonate, sodium sulfate, mixtures thereof, STP and mixtures of STP and sodium sulfate, said method comprising adding aqueous alkali metal nitrilotriacetate, containing from about 40% to about 70% by weight alkali metal nitrilotriacetate and having a temperature of from about 0°C to about 120°C, to an agitated bed of the inorganic salt, having an initial temperature of from about 300°C to about 550°C; sufficient aqueous nitrilotriacetate being added to cool the bed below about 300°C prior to dehydration of the bed and the addition of aqueous nitrilotriacetate and dehydration of the bed being complete at a bed temperature of at least about 160°C when STP is present or about 120°C when STP is not present.

2. The process of claim 1 wherein the aqueous alkali metal nitrilotriacetate has a temperature of 80° to 110°C.

3. The process of claim 1 wherein the inorganic salt has a temperature of from about 400°C to about 500°C.

4. The process of claim 1 wherein the aqueous alkali metal nitrilotriacetate contains 40 to 50% nitrilotriacetate.

5. The process of claim 1 wherein the inorganic salt is sodium tripolyphosphate.

6. The process of claim 1 wherein the alkali metal nitrilotriacetate is trisodium nitrilotriacetate.

\* \* \* \* \*